

July 21, 1925.

1,546,926

E. H. GAUGHAN

PROCESS OF MAKING POWDERED ZINC

Filed Aug. 17. 1921



Edward H. Gaughan  
By Hull, Brooks & West  
Attns.

## UNITED STATES PATENT OFFICE.

EDWARD H. GAUGHAN, OF CLEVELAND, OHIO.

## PROCESS OF MAKING POWDERED ZINC.

Application filed August 17, 1921. Serial No. 492,924.

*To all whom it may concern:*

Be it known that I, EDWARD H. GAUGHAN, a citizen of the United States, residing at Cleveland, in the county of Cuyahoga and State of Ohio, have invented a certain new and useful Improvement in Processes of Making Powdered Zinc, of which the following is a full, clear, and exact description, reference being had to the accompanying drawings.

This invention relates to a process of making powdered or finely divided zinc, and has for its general object to increase very greatly the rate of production thereof as well as the proportion of zinc obtainable in such powdered or pulverized form from a given quantity of the molten metal. I accomplish these general objects in and through the process herein described and by means of an apparatus shown in the drawings forming part hereof, wherein Fig. 1 represents a diagrammatic longitudinal sectional view through such apparatus; and Fig. 2 a sectional elevation of the pulverizing or atomizing nozzle.

Describing first the apparatus referred to, 1 denotes generally a furnace for the melting of the zinc, said furnace supporting therein a crucible 2 and having beneath and surrounding the said crucible, a combustion chamber 3 with which there communicates a suitable fluid fuel burner 4, the furnace being provided with an outlet flue 5 leading from the upper portion thereof.

At the right of the furnace 1 there is shown a collecting chamber 6 for the atomized or powdered zinc, this collecting chamber having a bottom 7 inclined downwardly from its receiving end toward its delivery end and provided at such delivery end with an outlet adapted to discharge the powdered zinc into a suitable receptacle 9.

As a means for atomizing the molten zinc in the crucible 2, I preferably employ the following construction:—10 denotes a pipe the lower end of which extends into, and in close proximity to the bottom of, the crucible, being spaced above such bottom a sufficient distance to enable the impurities present in an ordinary run of the zinc to rest upon the bottom without building up to a sufficient height to be drawn out through the said pipe. The pipe 10 is bent toward the chamber 6 and is connected by a coupling 11 with the inner tubular member 12 of

the atomizer, which is in the form of an injector. This tubular member 12 has its front or delivery end 12<sup>a</sup> flared outwardly toward a surrounding sleeve member 13, which is threaded into the front end of a T-casing 14. The rear end of the member 12 is connected to the rear end of said T-casing by means of a sleeve 15, which is threaded onto the said member and into the rear end of said casing, being provided at its rear end with recesses 15<sup>a</sup> for the application of a suitable tool. The central branch 16 of the T-casing has threaded thereinto a coupling 17 which carries the delivery end 70 of a supply pipe for compressed air, indicated at 18.

With the parts constructed and arranged as described, my process will be realized in the following manner:—The zinc which is melted in the crucible 2 will be drawn through the pipe 10 and through the delivery end 12<sup>a</sup> of the inner member 12 of the injector or atomizer by the air passing about the delivery end of said member through the surrounding sleeve member 13. In order to prevent the solidification of the molten zinc prior to its atomization, the air supplied through the pipe 18 should have a temperature of about 800° F., or somewhat higher. Flaring the outer end of the inner member 12 restricts the passageway 19 provided between such end and the surrounding sleeve and thus facilitates the atomization of the zinc, as will be pointed out hereinafter.

It will be noted that the outer end of the sleeve member 13 projects beyond the corresponding end 12<sup>a</sup> of the inner member 12. This arrangement of parts results in very finely subdividing the molten zinc. If, however, the inner member 12 projects beyond the outer member 13, the zinc is subdivided into relatively coarse particles. By adjusting the positions of the delivery ends of the members 12 and 13, corresponding variations in the fineness of the zinc particles is secured.

In the practice of my process I have used a three-quarter inch pipe for the inner member 12 and an inch and a quarter threaded sleeve for the outer member 13. By flaring the end of the inner member outwardly, as shown at 12<sup>a</sup>, a space about one-eighth inch in width will be provided between the delivery end of the inner member and the surrounding member 13. With a small delivery opening for the zinc, air will be em-

ployed under a pressure as high as 80 pounds per square inch. With a larger delivery opening, produced by the outwardly flaring end 12<sup>a</sup> of the inner injector member, a lower air pressure may be employed—say about 30 pounds per square inch; and, with this low pressure, a very fine subdivision of the zinc is accomplished.

The pulverized or powdered zinc is delivered upon the inclined floor 7 and thence may be conducted by gravity or by any appropriate movable device to the outlet opening 8.

By the practice of my process I am enabled greatly to increase the rapidity of manufacture of the powdered zinc; also greatly to increase the efficiency of the operation, converting from 90% upward of the molten zinc into the powdered or pulverized form.

Having thus described my invention, what I claim is:

1. The process of powdering or pulverizing zinc which consists in conducting molten zinc through a tube and to the delivery end of the latter by means of an injector having a delivery portion surrounding the delivery end of said tube and to which a heated fluid under pressure is supplied, and varying the relative positions of the delivery ends of the

tube and injector thereby to vary the size of the zinc particles.

2. The process of powdering or pulverizing zinc which consists in conducting molten zinc through the inner member of an injector having its delivery end outwardly flared, by means of a heated fluid under pressure supplied to the outer member of such injector.

3. The process of powdering or pulverizing zinc which consists in delivering molten zinc in an outwardly flaring direction from the delivery end of the inner member of an injector, into a heated fluid under pressure passing through the outer member of such injector and surrounding such delivery end, whereby the zinc will be atomized.

4. The process of powdering or pulverizing zinc which consists in delivering molten zinc in an outwardly flaring direction from the delivery end of the inner member of an injector, into a heated fluid under pressure passing through the outer member of such injector and surrounding such delivery end, and varying the relative positions of the delivery ends of said members, thereby to vary the size of the zinc particles produced.

In testimony whereof, I hereunto affix my signature.

EDWARD H. GAUGHAN.